

Dec. 8, 1953

A. P. GAGNEBIN ET AL

2,662,011

ABRASION AND CORROSION RESISTANT WHITE CAST IRON

Filed Aug. 20, 1951



*Fig. 1.*



*Fig. 2.*



*Fig. 3.*



*Fig. 4*

ALBERT PAUL GAGNEBIN  
LESLIE LOUIS SEIGLE  
INVENTORS

*BY  
A. Dr. Weller*  
ATTORNEY

## UNITED STATES PATENT OFFICE

2,662,011

ABRASION AND CORROSION RESISTANT  
WHITE CAST IRON

Albert Paul Gagnebin, Red Bank, N. J., and Leslie Louis Seigle, Dorchester, Mass., assignors to The International Nickel Company, Inc., New York, N. Y., a corporation of Delaware

Application August 20, 1951, Serial No. 242,722

8 Claims. (Cl. 75—128)

1

The present invention relates to nickel-chromium alloy white cast irons and more particularly to nickel-chromium alloy white cast irons having a very fine grain structure and possessing an improved combination of strength, wear or abrasion resistance and corrosion resistance.

Heretofore, the art has endeavored to employ alloy white cast irons in applications where wear or abrasion resistance were required of these materials. However, it has been found that prior art alloy white cast irons frequently lacked a satisfactory combination of strength, toughness, corrosion resistance and wear resistance, particularly in applications such as oil well pump parts. Furthermore, in applications requiring toughness and corrosion resistance, the prior art has been accustomed to employ austenitic nickel, nickel-chromium or nickel-copper-chromium gray cast irons. It has been found that such materials, although possessing a satisfactory degree of corrosion resistance and toughness, frequently lack the necessary wear or abrasion resistance required in many applications. Another type of cast iron employed in the foregoing and analogous applications by the prior art is the high-chromium white cast iron containing, for example, 25% chromium. Although such materials are satisfactory in many applications, they do not resist corrosive attack by strong caustics and suffer the serious disadvantage that they cannot be melted in the cupola furnace, which is a furnace commonly employed in cast iron foundries and one which is the foundryman's most economical melting tool. Thus, a demand has existed in the art for a cast iron which would offer a satisfactory combination of wear resistance, corrosion resistance and strength together with the capacity of being readily melted in the cupola.

In addition to the foregoing, there are many applications, such as in rolling mill rolls and the like, wherein a cast iron roll having a very fine-grain structure which will not "watermark" soft metals, e. g., copper, aluminum, etc., and having adequate strength for such service, is desired.

Although many attempts were made to overcome the foregoing difficulties and other difficulties and to provide a cast iron having a satisfactory combination of wear or abrasion resistance, strength, fine-grained structure and corrosion resistance, none, as far as we are aware, was entirely successful when carried into practice commercially on an industrial scale.

It has now been discovered that a nickel-chromium-silicon alloy white cast iron provides

2

an improved and useful combination of fine-grain structure, wear resistance, corrosion resistance, hardness, strength and toughness when the alloy compositions are maintained within certain critical limits and within a critical relationship as defined hereinafter, and that this iron can be melted readily in a cupola.

It is an object of the present invention to provide a new alloy white cast iron having a very fine-grain structure even in heavy sand cast sections.

Another object of the invention is to provide a new alloy white cast iron having a microstructure wherein the carbide phase occurs as the dispersed phase.

The invention also contemplates providing a new alloy white cast iron having an improved combination of wear or abrasion resistance, strength, hardness and corrosion resistance as compared to prior art alloy white cast irons.

It is a further object of the invention to provide a new alloy white cast iron having very high chilling propensity and which can readily be melted in the cupola.

The invention further contemplates providing a new white cast iron roll for rolling soft metals, such as aluminum, etc., which will provide a bright finish thereon and which will not "watermark" the soft metals.

Other objects and advantages will become apparent from the following description taken in conjunction with the accompanying drawings in which:

Figure 1 is a reproduction of a photomicrograph taken at 25 diameters of a prior art alloy white cast iron;

Fig. 2 depicts a reproduction of a photomicrograph taken at 25 diameters of an alloy within the scope of the invention;

Fig. 3 shows a reproduction of a photomicrograph taken at 500 diameters of an alloy within the scope of the present invention; and

Fig. 4 is a reproduction of a photomicrograph taken at 500 diameters of a special and preferred alloy within the scope of the present invention.

Generally speaking, the present invention contemplates an alloy white cast iron containing about 3% to about 3.7% carbon, about 0.5% to about 3% silicon, about 4% to about 8% nickel, about 4% to about 15% chromium, about 0.2% to about 1.5% manganese and the balance essentially iron including small amounts of impurities, e. g., phosphorus and sulfur in the amounts usually found in cast iron, i. e., in amounts not over about 0.4% and about 0.15%, respectively. Not

more than about 0.2% carbon is present in the uncombined form. It has been found that in order to obtain the improved combination of fine-grain structure, strength, hardness, abrasion resistance, corrosion resistance, wear resistance, high chilling propensity, etc., which characterize alloys within the scope of the invention, the carbon, nickel, chromium and silicon contents must be controlled according to the following relation:

$$\frac{\% \text{ Carbon} + \frac{\% \text{ Nickel}}{28}}{24} + \frac{\% \text{ Chromium} + \frac{\% \text{ Silicon}}{4}}{4} = 4.2 \text{ to } 5.0$$

The microstructure of alloys made according to the invention is comprised of a carbide phase and an austenite-martensite phase. The ratio of austenite to martensite in the austenite-martensite phase varies according to the section size, the silicon content, etc., as will be readily appreciated by those skilled in the art.

Alloys of the invention are characterized by a very fine-grain structure even in heavy sections, by high dispersal of the microstructural constituents and by freedom from gross dendritic constituents. It is believed that the fine-grain structure contributes importantly to the unusual combination of properties possessed by the alloy, and this fine-grain structure, together with the high strength of the alloy, enables the use of the alloy in applications where a coarse structure is undesirable, e. g., rolling mill rolls for soft metals, etc. Among the unusual and high properties possessed by the alloy are high strength, toughness, a high combination of corrosion and wear resistance, resistance to thermal shock, uniform and high hardness even in heavy sand cast sections, high chilling propensity, etc.

This unusual combination of properties is obtained when the compositions are controlled within the foregoing ranges, particularly when the carbon content is controlled according to the relationship set forth hereinbefore. The carbon content should be within the range of about 3% to about 3.7% to provide a critical amount of carbide dispersed in an austenite-martensite matrix. The hardness decreases at lower carbon contents and undesirable carbide needles occur at high carbon contents. The silicon content is controlled within the range of about 0.5% to about 3% to prevent excessive austenite formation which occurs when the silicon is below about 0.5% and to prevent formation of pearlite and a weakening effect which occurs above about 3% silicon. Silicon has an important effect upon the properties obtained in alloys of the invention and can be used to control the proportion of austenite to martensite in the austenite-martensite phase, inasmuch as increases in the silicon content increase the proportion of martensite. When the nickel is below 4% undesirable pearlite formation occurs and when the nickel is above about 8% excessive austenite is retained. Similarly, when the chromium is below 4% the desired fine distribution of carbide is not obtained and when chromium exceeds about 15% a detrimental effect is encountered which is believed to be associated with ferrite formation. Control of the manganese content is important inasmuch as below about 0.2% inadequate control of sulfur distribution is obtained and above about 1.5% an excessive amount of austenite is formed.

As pointed out hereinbefore, a feature characterizing alloys of the invention is the exceptionally fine-grain structure found therein. This

feature is illustrated by the attached Figs. 1 and 2 of the drawing. Fig. 1 is a reproduction of a photomicrograph depicting the microstructure at 25 diameters of an alloy white cast iron containing about 1.5% chromium and about 4.5% nickel (such as is sold under the trade-mark "Ni-Hard"). The light-colored phase appearing in the microstructure of the aforesaid alloy is a massive carbide phase. Fig. 2 is a reproduction

of a photomicrograph depicting the microstructure, at the same magnification as Fig. 1, of an alloy of the invention. As illustrated by Fig. 2, the carbides in alloys of the invention appear as a fine, well-dispersed phase contrasting sharply to the massive appearance of the carbides of Fig. 1. Figs. 1 and 2 represent the structures of the aforesaid alloys at the center of 3½ inch sand cast sections, and the specimens from which the aforesaid figures were obtained were etched to darken the austenite-martensite phase but not the carbide phase.

Within the range of alloy compositions contemplated by the invention, and set forth hereinbefore, a special (and preferred) alloy having other advantages is obtained. This special alloy contains at least about 6.8% and up to about 10% or even about 15% chromium, with carbon, nickel, silicon, manganese, etc., within the ranges set forth hereinbefore and with the carbon, nickel, chromium and silicon contents controlled in accordance with the relationship set forth hereinbefore. The aforesaid special alloy incorporates the unexpected and unusual discovery that when the chromium content of the alloy is within the aforesaid range, a microstructure which is the complete reverse of the microstructure normally encountered in white cast irons is obtained. Thus, normal alloy white cast irons are characterized by a microstructure wherein the continuous phase is a massive carbide phase and the remainder of the structure is a discontinuous phase usually comprising martensite and austenite. In the aforesaid special alloy of the invention, however, a martensite-austenite phase is the continuous phase and the primary carbides are dispersed therethrough in a discontinuous manner. This unusual reversal in microstructural constituents is clearly illustrated by Figs. 3 and 4 of the drawing. Fig. 3 is a reproduction of a photomicrograph at 500 diameters depicting the structure at the center of a 3½ inch sand cast section of an alloy within the invention and containing about 6% nickel and about 6% chromium. Fig. 4 is a reproduction of a photomicrograph depicting the microstructure, at the same magnification as Fig. 3, found at the center of a similar casting made from a preferred alloy within the invention and containing about 6% nickel and about 8% chromium. It will be noted that the carbides found in Fig. 4 are dispersed discontinuously in a continuous austenite-martensite matrix, and that there is marked refinement of the structure as compared to Fig. 3.

In the special compositions wherein the reversal in matrix constituents occurs when the chromium equals or exceeds about 6.8%, a nickel content of at least about 4% is required as otherwise the aforesaid reversal in microstructural constituents does not occur even with chromium contents of about 6.8% or more. The nickel content of the special composition should not exceed about 8%, as otherwise excessive amounts of austenite are formed and the alloy becomes relatively soft.

In addition to the amounts of carbon, nickel,

chromium and silicon disclosed hereinbefore, all the alloys made in accordance with the invention may contain the usual impurities in the amounts usually found in white cast iron. For example, amounts of sulfur up to about 0.15%, e.g., 0.02% to 0.15%; and of phosphorus up to about 0.4%, e.g., 0.02% to 0.4%, may be present without harmfully affecting the properties of alloys made according to the invention. Furthermore, other metallic elements, such as copper, molybdenum, etc., commonly found in white cast irons, may be present in alloys of the invention in small amounts up to about 2%, e.g., 0.1% to 2%, and in small amounts up to about 1%, e.g., 0.1% to 1%, respectively, without detrimental results; although not more than a total of about 3% of these elements should be present. These elements may be considered as replacing part of the iron content of the alloy, and when, in defining the composition of the alloy, it is stated that the balance is essentially iron, or the balance is iron, it is not intended to exclude the aforesaid impurities and metallic elements, since the alloys of the invention are essentially the same in properties regardless of the presence or absence of the foregoing impurities and metallic elements in the amounts set forth hereinbefore.

Alloys having the aforesaid unusual combination of properties and made according to the invention are characterized by a very fine grain-size and a uniform high hardness even in heavy sand cast sections. In addition, chill castings made of the alloy have a very fine-grain structure as compared to other chill cast alloy white irons; high chilling propensity, high strength and toughness.

In order to give those skilled in the art a better appreciation of the advantages of the invention, illustrative compositions and sand cast properties of certain white iron castings are set forth in Tables I and II, respectively.

Table I.—Composition<sup>1</sup>

| Alloy No. | Percent C | Percent Si | Percent Ni | Percent Cr | Percent Mn | Percent S | Percent P |
|-----------|-----------|------------|------------|------------|------------|-----------|-----------|
| 1         | 2.6       | 1.0        | 6.0        | 6.0        | 0.5        | 0.1       | 0.1       |
| 2         | 3.6       | 0.9        | 5.7        | 5.7        | 0.6        | 0.1       | 0.1       |
| 3         | 3.5       | 1.8        | 5.6        | 5.6        | 0.6        | 0.1       | 0.1       |
| 4         | 3.5       | 1.8        | 5.4        | 7.1        | 0.6        | 0.1       | 0.1       |
| 5         | 3.7       | 2.2        | 6.1        | 7.9        | 0.5        | 0.03      | 0.03      |

<sup>1</sup> Balance iron.

Table II.—Sand cast properties

| Alloy No. | Transverse props. <sup>1</sup> |                 | Izod impact, ft.-lbs. | BHN |
|-----------|--------------------------------|-----------------|-----------------------|-----|
|           | Load, lbs.                     | Deflection, in. |                       |     |
| 1         | 4,810                          | 0.11            | 35                    | 375 |
| 2         | 3,800                          | 0.07            | 23                    | 555 |
| 3         | 4,680                          | 0.08            | 21                    | 616 |
| 4         | 5,080                          | 0.10            | 24                    | 600 |
| 5         | 5,300                          | 0.10            | 30                    | 540 |

<sup>1</sup> Obtained on 1.25-inch diameter arbitration bar over 12-inch centers.

From the data in Tables I and II, it may be seen that alloy No. 1, an alloy outside the scope of the present invention, had the low sand cast hardness of only 375 Brinell, whereas alloy No. 2, having essentially the same base composition as alloy No. 1, but having a carbon-nickel-chromium-silicon relationship as required by the invention and as set forth hereinbefore, had a sand cast hardness of an entirely different and higher

order in the same section size as alloy No. 1, i.e., a hardness of 555 Brinell. It may be noted from Tables I and II that alloys No. 4 and No. 5, special alloys within the scope of the invention having the reversed structure discussed hereinbefore; i.e., a microstructure wherein the carbides are dispersed discontinuously in an austenite-martensite matrix, possess an improved combination of properties as compared to alloys Nos. 2 and 3 which represent less preferred alloys within the scope of the invention. As an illustration of the high hardness provided in heavy sections sand cast in the alloy provided by the present invention, a step bar casting in alloy No. 2 exhibited a hardness of 550 Brinell in the  $\frac{1}{2}$ -inch section; 578 Brinell in the 1-inch section and 590 Brinell in both the 2-inch and 4-inch sections.

As indicated hereinbefore, chill castings of the alloys of the invention also possess improved properties. For example, a 1.2-inch diameter arbitration bar chill cast in alloy No. 1 (which, as pointed out hereinbefore, is outside the present invention) had a hardness of 418 Brinell, whereas a similar arbitration bar chill cast in alloy No. 2 (which is within the present invention) had a hardness of 564 Brinell. This significant increase in hardness found in alloy No. 2 as compared to alloy No. 1 was accompanied by increases in transverse strength and in toughness. Chill blocks of alloys Nos. 2 and 3 measuring 6" x 6" x 2" cast against a chiller on one of the 6" x 2" faces were completely white and had hardnesses at the chill face of 725 to 744 Brinell and 719 to 744 Brinell, respectively. These chill castings had a very fine-grain structure.

As illustrated by comparing Fig. 4 with Fig. 3, the microstructure of special alloys of the invention is unexpectedly fine even as compared to other alloys within the invention but containing less than the preferred amount of at least 6.8% chromium. This discovery is believed due to the dispersal of the carbide phase in a continuous austenite-martensite matrix which has been found to occur in special alloys of the invention. Those skilled in the art will appreciate that the continuous austenite-martensite matrix of the preferred alloy provides a tougher product having improved resistance to thermal and mechanical shock, as compared to less preferred alloys of the invention having a continuous carbide network structure.

Preferred alloys made according to the invention have improved strength and toughness when compared to the commonly used white cast irons containing about 1.5% chromium and 4.5% nickel (such as are sold under the trade-mark "Ni-Hard"). For example, when tested in the form of 1.2-inch diameter sand cast arbitration bars, preferred alloys of the invention are about 30% stronger in the transverse test and about 20% tougher in the impact test than the commonly used 1.5% chromium-4.5% nickel white cast irons. In addition, the alloys of the invention provide superior properties in the chill cast condition to alloys of the commonly used 1.5% chromium-4.5% nickel white cast irons. The improved sand cast strength found in preferred alloys of the invention, as compared to prior art alloy white cast irons, provides the great practical advantage over such materials that articles having an intricate shape, etc., which are difficult to cast in a chill mold, may now be cast satis-

factorily in sand molds when the alloy of the invention is employed.

Corrosion tests conducted in aerated dilute 5% sulfuric acid and in aerated simulated mine water (0.8% ferric sulfate) show that the new materials have superior corrosion resistance as compared to the commonly used 1.5% chromium-4.5% nickel white cast irons. For example, sand cast corrosion test specimens in the commonly used 1.5% chromium-4.5% nickel white cast irons corroded about 2.2 times faster than sand cast specimens of the new material when tested in aerated dilute sulfuric acid and about 20% faster when tested in aerated simulated mine water.

Field tests in handling abrasive materials, such as blasting shot, etc., have shown that alloys within the invention have excellent resistance to abrasion or wear and are comparable in this respect to the commonly used 1.5% chromium-4.5% nickel white cast irons. It is believed that the fine dispersal of carbides found in alloys of the invention contributes importantly to the good wear resistance thereof.

The present invention is particularly applicable to castings requiring an improved combination of fine-grained structure, strength, hardness, wear resistance, and corrosion resistance not provided by alloy white cast irons heretofore commonly used in the art. For example, oil well pump parts used in pumping abrasive and corrosive crudes may advantageously be made from the alloy of the invention. Highly stressed components, such as parts for gyratory crushers, grinding mill roll heads, stamp shoes or crusher teeth also provide another application for the new material. A particularly suitable application for the new alloy and one where the fine grain thereof is particularly useful is in rolls used for rolling soft metals, such as aluminum, etc., where the "watermark" produced on such metals by prior art cast iron rolls is minimized or eliminated due to this extremely fine grain. Among the other applications of the new material are the following: grizzly discs, rabble arms, clay augers, dredging equipment, sludge pumps, valve seats, impellers, etc.

The special white cast iron compositions contemplated by the present invention can be melted in the usual foundry melting equipment employed for melting alloy white cast iron, e. g., the direct or indirect arc furnace, the induction furnace, fuel-fired melting furnaces (such as the air furnace), etc. A special feature of the white cast irons provided by the invention is that they may readily be melted in the cupola furnace.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

We claim:

1. As a new article of manufacture, a white iron casting having included sections at least about one-half inch in thickness and being characterized by a fine-grain structure by a microstructure containing a primary massive carbide phase dispersed in a discontinuous manner throughout a continuous martensite-austenite phase and containing about 3% to about 3.7% carbon, about 0.5% to about 3% silicon, about 4%

5 to about 8% nickel, about 6.8% to about 15% chromium, the carbon, silicon, nickel and chromium being present in such amounts as will satisfy the relationship expressed in the equation

$$\% C + \frac{\% Ni}{28} + \frac{\% Cr}{24} + \frac{\% Si}{4} = 4.2 \text{ to } 5.0$$

about 0.2% to about 1.5% manganese, and the balance substantially all iron.

2. A casting having included sections at least about one-half inch in thickness comprised of a white cast iron containing about 3.0% to about 3.7% carbon, about 0.5% to about 3% silicon, about 4% to about 8% nickel, about 6.8% to about 10% chromium, the carbon, silicon, nickel and chromium contents being so related to each other that the sum of the percentage of carbon plus the percentage of nickel divided by 28 plus the percentage of chromium divided by 24 plus the percentage of silicon divided by 4 lies between 4.2 to 5.0 inclusive, about 0.2% to about 1.5% manganese and the balance substantially all iron, said casting being characterized by a very fine-grain structure and by a microstructure containing a discontinuous primary carbide phase dispersed through a continuous martensite-austenite phase.

3. A casting having included sections at least about one-half inch in thickness comprised of a martensitic white cast iron containing about 3.0% to about 3.7% carbon, about 0.5% to about 3% silicon, about 4% to about 8% nickel, about 4% to about 15% chromium, the amounts of carbon, silicon, nickel and chromium present in any given alloy being further limited in that their respective amounts must fall within the range allowed by the equation

$$\% C + \frac{\% Ni}{28} + \frac{\% Cr}{24} + \frac{\% Si}{4} = 4.2 \text{ to } 5.0$$

about 0.2% to about 1.5% manganese and the balance substantially all iron, said casting being characterized by a very fine-grain structure.

4. As a new article of manufacture, a white cast iron roll characterized by a fine-grained structure and by a microstructure containing a discontinuous massive carbide phase dispersed throughout a continuous martensite-austenite phase and containing about 3% to about 3.7% carbon, about 4% to about 8% nickel, about 6.8% to about 15% chromium, about 0.2% to about 1.5% manganese, with the balance essentially iron, and with the carbon, silicon, nickel and chromium being correlated according to the relationship:

$$\% C + \frac{\% Cr}{24} + \frac{\% Ni}{28} + \frac{\% Si}{4} = 4.2 \text{ to } 5.0$$

5. As a new article of manufacture, a white cast iron roll characterized by a fine-grained structure and by a microstructure containing a discontinuous massive carbide phase dispersed throughout a continuous martensite-austenite phase and containing about 3% to about 3.7% carbon, about 4% to about 8% nickel, about 6.8% to about 10% chromium, about 0.2% to about 1.5% manganese, with the balance essentially iron, and with the carbon, silicon, nickel and chromium being correlated according to the relationship:

$$\% C + \frac{\% Cr}{24} + \frac{\% Ni}{28} + \frac{\% Si}{4} = 4.2 \text{ to } 5.0$$

6. As a new article of manufacture, a white cast iron roll characterized by a fine-grained structure and containing about 3% to about

3.7% carbon, about 4% to about 8% nickel, about 4% to about 15% chromium, about 0.2% to about 1.5% manganese, with the balance essentially iron, and with the carbon, silicon, nickel and chromium being correlated according to the relationship:

$$\% C + \frac{\% Cr}{24} + \frac{\% Ni}{28} + \frac{\% Si}{4} = 4.2 \text{ to } 5.0$$

7. The method of producing a martensitic alloy white cast iron which comprises establishing a cast iron bath containing about 3% to about 3.7% carbon, about 0.5% to about 3% silicon, about 4% to about 8% nickel, about 4% to about 15% chromium, about 0.2% to about 1.5% manganese and the balance essentially of iron, adjusting the composition of said bath such that the chromium, silicon and nickel contents are correlated with the carbon content of said bath according to the relationship:

$$\% C + \frac{\% Cr}{24} + \frac{\% Ni}{28} + \frac{\% Si}{4} = 4.2 \text{ to } 5.0$$

and thereafter casting said cast iron bath to obtain a martensitic white cast iron casting having included sections at least about one-half inch in thickness and characterized by a very fine-grain structure.

8. The method of producing a martensitic alloy white cast iron which comprises establishing a

cast iron bath containing about 3% to about 3.7% carbon, about 0.5% to about 3% silicon, about 4% to about 8% nickel, about 6.8% to about 15% chromium, about 0.2% to about 1.5% manganese and the balance essentially of iron, adjusting the composition of said bath such that the chromium, silicon and nickel contents are correlated with the carbon content of said bath according to the relationship:

$$\% C + \frac{\% Cr}{24} + \frac{\% Ni}{28} + \frac{\% Si}{4} = 4.2 \text{ to } 5.0$$

and thereafter casting said cast iron bath to obtain a martensitic white cast iron casting having included sections at least about one-half inch in thickness and characterized by a very fine-grain structure and by a microstructure containing a discontinuous primary carbide phase dispersed throughout a continuous martensite-austenite phase.

ALBERT PAUL GAGNEBIN.  
LESLIE LOUIS SEIGLE.

References Cited in the file of this patent

UNITED STATES PATENTS

| Number    | Name        | Date          |
|-----------|-------------|---------------|
| 1,988,912 | Merica      | Jan. 22, 1935 |
| 2,189,131 | Cape et al. | Feb. 6, 1940  |